

## [54] METHOD FOR THE TREATMENT OF TEXTILE FIBRES

[75] Inventors: Ryo Umebara; Fujio Bekku, both of Ichinomiya, Japan

[73] Assignee: I.W.S. Nominee Company Limited, London, England

[22] Filed: May 16, 1972

[21] Appl. No.: 253,797

## [30] Foreign Application Priority Data

May 20, 1971 Japan..... 46-83636

[52] U.S. Cl. .... 28/72.17, 8/128 A, 28/75 WT

[51] Int. Cl. .... D02g 3/36, D02j 1/22

[58] Field of Search .. 28/72.1, 75 WT, 76 R, 72.17; 19/66 R; 8/127.6, 128 R, 128 A

## [56] References Cited

## UNITED STATES PATENTS

3,677,694 7/1972 Sugimoto et al. .... 8/128 A  
3,687,605 8/1972 Farmer ..... 8/128 A

## FOREIGN PATENTS OR APPLICATIONS

985,621 3/1965 Great Britain ..... 28/72.17

Primary Examiner—Louis K. Rimrodt

Attorney, Agent, or Firm—Harold L. Stowell

## [57] ABSTRACT

This specification discloses a method of crimping protein fibres by drafting. Untwisted fibres are treated with an aqueous solution of alcohol, which may optionally contain an acid and a setting agent for the protein fibres, such as formaldehyde. They are then drafted and are subsequently relaxed to form the crimps. The crimps can be set, for example by steam, with the help of the setting agent after processing and the fibres dried. The preferred alcohol and acids are those which will evaporate on drying, notably having boiling points below 120°C. The drafted fibres may be set without applied tension, and the resulting crimp waves set as mentioned above. Alternatively the drafted fibres may be set in tension and the fibres relaxed at a later stage to produce the crimps. They can be relaxed, for example, after conversion into yarn or fabric. The invention also provides apparatus in which the method can be carried out, a preferred feature being the use of a vacuum padding device which causes rapid and complete wetting of the fibres with the alcohol solution. The invention overcomes the disadvantages inherent in crimping conduct by drafting twisted fibres.

21 Claims, 3 Drawing Figures



PATENTED NOV 26 1974

SHEET 1 OF 3

3,849,848

FIG. 1



PATENTED NOV 26 1974

3,849,848

SHEET 2 OF 3



PATENTED NOV 26 1974

3,849,848

SHEET 3 OF 3

*Fig. 3*



**METHOD FOR THE TREATMENT OF TEXTILE FIBRES**

This invention relates to a method and apparatus for drafting non-twisted protein fibres to crimp them spontaneously.

Keratin fibres can be crimped in the form of top or carded sliver by a stuffer box method, in the form of top or yarn by the twist-draft-set-untwist method and in the form of yarn by the draft-release method.

In fibres crimped by the stuffer box method the curvature at certain positions in the crimped fibres is exceedingly sharp, and strain is concentrated in these sharply curved portions. As the fibres are steam set in such a configuration, the tensile strength of the fibres is greatly reduced. Steam-setting produces only a temporary set and when permanent set is required, chemical setting with inorganic or organic reducing agents is employed. Permanent setting further reduces the tensile strength and this causes problems in subsequent processing or in the quality of the final product.

In the twist-draft-set-untwist method and the draft-release method, the fibres are drafted mechanically and on release become twisted and crimped. However, twisting of fibres during the process inhibits the diffusion of aqueous solutions, water-vapour diffusion and heat transmission. In consequence, only the surface of the fibre bundle is wetted while the inside is hardly damp, and during drafting the surface layer of fibres is readily drafted while the inside layers are less efficiently drafted, so that uneven drafting inevitably results.

As highly drafted fibres are not the stable  $\alpha$ -type keratin fibres of natural wool, the fibres are severely damaged. When subjected to setting with boiling water, steam or chemical agents for permanently setting the crimp, the fibres are further damaged, and the tensile strength is further reduced. In methods involving twisting the fibres as described above, it becomes very difficult to dry them and it is uneconomical to untwist them.

A first aspect of the present invention relates to a method for crimping protein fibres by applying to the fibres an aqueous solution of an alcohol, drafting the fibres, and subsequently relaxing the fibres.

Non-twisted keratin fibres are preferably used in this invention. Keratin fibres include sheep's wool, mohair, alpaca, vicuna, llama, cashmere, and camel hair, and may be used in the form of carded sliver, tops and rovings of such fibres, which are non-twisted and arranged uniformly parallel along the fibre axis.

In the preferred practice of the invention, the fibres are well impregnated in an acid-containing or alkali-containing aqueous solution of an alcohol, which generally contains a high concentration of the alcohol, in order to render them draftable more readily and with a reduced energy. Keratin fibres are characterised by a 30 percent index; that is to say that when sheep's wool is drafted by 30 percent and then released, it recovers to the original state without any internal strain. The treated fibre when adequately dried shows the same tensile strength properties as untreated sheep's wool fibres. While the performance of the invention does not depend upon any theory as to its mode of operation, this phenomenon is understood to be due to the opening by water of the hydrogen bonds stabilising the polypeptide chain, which can be reversed on dry-

ing. Additionally there are other reversible bonds having the property of stabilising the polypeptide chain, such as salt bonds and hydrophobic bonds. The former bond is opened by adding acid or alkali and the latter bond is opened by an alcohol. Thus the drafting properties of sheep's wool and other keratin fibres can be further increased.

The impregnating media consisting of an acid-containing or alkali-containing aqueous solution of an alcohol should be removed in the subsequent drying process. If it is not removed substantially completely in the drying process it greatly reduces the strength of the fibres. The acids, alkalis and alcohols which are preferred are those having a similar volatility to water and preferably not having a boiling point higher than about 120°C. For the purposes of this invention, formic acid (b.p. 100.5°C) and acetic acid (b.p. 118°C) are the most preferred acids, ammonia (b.p. -33.35°C) the preferred alkali, and methanol (b.p. 64.7°C), ethanol (b.p. 78.3°C), n-propanol (b.p. 97.2°C), iso-propanol (b.p. 82.5°C), n-butanol (b.p. 117.7°C) and iso-butanol (b.p. 108°C) are the preferable alcohols, especially n-propanol and iso-propanol. The acid or alkali is added in such an amount as to make the pH of the aqueous solution strongly acidic or strongly alkaline. The concentration of the alcohol in water is normally at least 10 percent by volume and is preferably in the range 10-50 percent by volume.

Keratin fibres themselves are hydrophobic and if they are impregnated unevenly, the subsequent treatment is adversely affected. As the fibres should be impregnated evenly and rapidly it is desirable to replace the air surrounding the fibres quickly and completely by the impregnating liquid described above or its vapour. It is also desirable to allow the fibres to stand for a time after removal from the impregnating liquid to allow penetration of the impregnating liquor. Unless the fibres are allowed to stand for a sufficient time, they will subsequently be drafted unevenly and it will be difficult to obtain effective crimping.

The fibres treated in accordance with the invention do not have any twist and absorb the liquid much better than twisted fibres. Subsequent drying can be quickly performed, and untwisting is not required. Thus, processing becomes simplified. It is recommended to add simultaneously a small amount of thioglycollic acid, monoethanolamine sulphite, monothanolamine bisulphite or thiourea dioxide as a setting agent and formaldehyde (formalin, b.p. 96°C) as a cross-linking agent for crimp waves produced in a subsequent stage.

The length and the amount of drafting are determined in accordance with the subsequent crimping method. The fibres can be drafted by applying tension at two or more points along the advancing bundle of fibres, for example by using a pair of co-operating nip rollers one of which is driven faster than the other. When the fibres are drafted, crimped by removing tension, set without tension, and then dried, the number of crimps produced depends on the length of fibre bundle grasped between the points at which the drafting forces are applied (grasped length) and the amount of drafting of the fibres. When drafting with a grasped length shorter than the length of the individual fibres, the tension on the fibres increases and when the grasped length is longer than the individual fibres, the amount of fibre slippage increases. When a high tension is applied, fine crimp waves are produced, and when the

amount of fibre slippage is greater, so that a lesser tension is applied, large crimp waves are produced. Consequently, for obtaining optimum crimp waves, it is preferable to extend the fibres during drafting by 10 – 30 percent, and to apply drafting forces to the fibres at at least two points spaced apart by about the average fibre length.

When fibres are drafted and temporarily set under tension, and when after spinning the temporary set is removed to produce crimp, it is not recommended to draft highly. When highly drafted fibres are relaxed in the form of yarn, stress concentrates at points where the yarn twist is irregular and produces local hardness in the yarn. In such a case, therefore, it is preferable for the grasped length to equal the average fibre length and to draft moderately, i.e. by 5 – 20 percent.

The keratin fibres thus drafted are then set. When they are set without any applied tension, stress release rather than dimensional change is produced, but when they are set under tension, a dimensional change and not a stress release is produced. The results are opposite to each other and the setting conditions can be selected to produce the desired result.

When setting without tension (direct crimping method), fibres highly drafted by 10 – 30 percent as described above are released from tension to produce crimp waves, which can be set by steaming or boiling water, followed by drying to evaporate completely the previously absorbed liquid. When adding a setting agent, for example formaldehyde, linkages are introduced into the polypeptides to stabilize the molecular chains, and thus the crimp waves are fixed and set.

When being set under tension, (indirect crimping method) keratin fibres drafted moderately, i.e. by 5 – 20 percent as described above, can be steamed and dried under tension to evaporate the impregnating liquid and are set temporarily in the extended state. They can then be spun into yarn in a conventional manner and the fibres are relaxed when in the form of spun yarns or textile material made therefrom: that is, crimps are produced by treatment with steam, hot water or an impregnating liquid as described above. On drying to evaporate water of an impregnating solution the molecular chains again become stabilized, and there are obtained bulky yarns or textiles.

In the wool industry, fibres are usually allowed to stand for a long time for top ageing, and this represents a problem in the field. In the indirect crimping method, the period required for top ageing can be greatly shortened to produce end products having an attractive handle. If it is only desired to speed up top ageing the amount of drafting should be selected to be just enough to remove the natural crimp waves of the fibre, preferably less than about 10 percent. In this method, the drawing process can be performed quickly and continuously and the method is very advantageous.

The invention further provides an apparatus suitable for carrying out the method described above, which comprises means for impregnating the fibres with an aqueous solution of an alcohol, preferably containing at least 10 percent by volume of the alcohol, means for storing the impregnated fibres to allow penetration of the solution, means for drafting the fibres and means for setting and drying the fibres. The means for impregnating the fibres may be a conventional pad mangle or preferably a vacuum pad mangle. The drafting means can comprise at least two pairs of nip rollers, at least

the second pair being driven at a surface speed faster than the first pair. If there are three pairs of nip rollers, the third pair can be driven at the same surface speed as the second pair, whereby drafting forces imposed on the fibres between the first and second pair of rollers are retained between the second and third pair or, alternatively, the third pair can be driven at a lower surface speed whereby the drafting forces are released and crimps form in the fibres. The apparatus can further comprise a crimping chamber, a drying chamber provided with means for forwarding the fibres, for example a pair of belts which in one position can co-operate and maintain the drafting forces on the fibres, and a cooling device.

One example of the apparatus is shown in the attached drawings and the method and the apparatus of this invention will be more particularly described hereinafter with reference to the drawings, in which:

FIG. 1 shows a preferred device for completely impregnating or wetting keratin fibres in or by an impregnating liquid.

FIG. 2 shows apparatus for carrying out the process of this invention and incorporates the device of FIG. 1.

FIG. 3 is a photographic showing of crimped Australian merino wool as set forth in Example 1.

The device A shown in the drawings may be termed a vacuum padder and is composed of rollers 1 to 6 arranged to form a hexagonal section. Two of the rollers 2 and 5 are smaller than the others. At either end of the six assembled rollers pressure plates 7 and 8 are attached to form a closed space 9 on the inside.

Small rollers 10, 11, 12 and 13 are arranged in pairs above and below the main roller assembly. Endless mesh belts 14 and 15 span round the rollers 1, 2 and 3 and the small rollers 10 and 12 on the left hand side and around the rollers 4, 5 and 6 and the small rollers 11 and 13 in the right hand side of the drawing respectively. The belts introduce keratin fibres W to be processed and prevent them from winding into the rollers.

A liquid-supplying and discharging device and an exhaustion device are arranged outside the rollers. A tank 16 of an impregnating liquid, is connected with a closed tank 19 by way of a control cock 17 and a pipe 18. A flexible pipe 20 and a flexible pipe 21 are disposed between the pipe 18 and the lower part of the closed space 9 and between the closed tank 19 and the upper part of the closed space, respectively. To the root of the pipe 21, an exhaustion pipe 22 is attached, and is connected with a vacuum pump. A cock 23 is disposed under the closed tank 19.

In operation, an impregnating liquid is introduced into the tank 16, at which time the cocks 17 and 23 are shut. Then the cock 17 is opened to introduce the liquid through the pipes 18 and 20 into the lower part of the closed space 9 to fill it, as shown at 24. The liquid is also introduced to the closed tank 19. The air is exhausted from the pipe 22 to reduce the pressure in the closed space 9, which becomes saturated with vapour of the liquid. The liquid is an acid- or alkali-containing aqueous solution containing 10–50 percent by volume alcohol; its pH is adjusted to 1.0 – 4.0 or 9.0 – 11.0, and 0.5 – 5.0 percent formalin and thioglycollic acid, monoethanolamine sulphite or bisulphite, or thiourea dioxide may be added.

Non-twisted keratin fibres **W** are introduced from the upper side into the closed space **9** by the two endless mesh belts **14** and **15**, and pass downwardly through the impregnating liquid **24** retained in the nip between rollers **1** and **6**. The closed space **9** is kept under reduced pressure (about 100–760 mm Hg) by the pressure-reducing means described above. In the space above the liquid the air in the interstices between the fibres is quickly replaced by the vapour saturated with the impregnating liquid, and then the fibre is padded in the liquid. By this means the keratin fibres can be quickly and uniformly wetted. The fibres are passed between the rollers **1** and **6** to be squeezed to 50–100 percent wet pick up.

In the apparatus of FIG. 2, a U-type duct storage chamber **B** is positioned under the vacuum padder **A**, and there are further provided a drafting chamber **C**, a steaming chamber **D**, a drying chamber **E** and a cooler **F**. The drafting chamber, the steaming chamber and the drying chamber form a single assembly packed in a closed unit **26**, divided by walls **25** and **25'**. The keratin fibres **W** which have been passed through the padder **A** to improve their drafting properties, are passed through the storage duct **B** and the chambers **C**, **D** and **E** and finally pass over the cooler **F**.

The inlet arm of the U-type storage duct **B** is positioned under the padder, and the outlet arm is under the drafting chamber **C**. In the horizontal part of the duct **B**, two rollers **27** and **28** are provided and an endless mesh belt **29** spans them. The outer wall **30** of the duct is double, and the inside of the double wall is maintained at 20°–25°C by passing cooling water through pipes **31** and **32** and is closed tightly from the ambient air.

In the drafting chamber **C**, the fibre bundle **W** passes upwardly over forwarding rollers **33**, **34** and **35**, which control the applied loading tension, and then passes over rollers **36** and **37** which are disposed horizontally. Three co-operating pairs of grip rollers **38**, **39** and **40**, are arranged horizontally for drafting the fibres and their distance apart and the surface speed rate can be adjusted to any suitable value.

In the subsequent steaming chamber **D**, an endless mesh belt **44** passes over rollers **41**, **42** and **43** so as to forward the fibres **W** at the same level as that in the drafting chamber. Above the rollers, a little apart from them, an endless mesh belt **48** similarly passes over rollers **45**, **46** and **47** and the distance of the assembly from the lower roller is adjustable. In carrying out the direct crimping method, the latter belt and the rollers are positioned as shown by solid lines, and for the indirect crimping method they are lowered to the position shown by broken lines **50** so as to maintain the tension on the fibres, and the fibres are given tension by both endless belts **44** and **48**. A plurality of small rollers are provided over which the belts **44** and **48** pass so as to be tensioned satisfactorily. A steam jet is directed against the fibres passing over the belt **44** by means of a pipe **50** provided with many jet holes disposed adjacent to the spaces between the rollers **41**, **42** and **43**. A pipe **51** is additionally positioned under the chamber through which steam can be introduced from an external source to keep the temperature in the chamber **D** in the range 80°–125°C.

The subsequent drying chamber **E** is similar to the setting chamber **D**. In the drawing, the parts similar to those in the chamber **D** are shown by the same numer-

als with an added prime. The steam jet pipe **50** is omitted. The chamber is kept at a temperature in the range of 80°–110°C.

The chambers are divided by walls **25**, **25'** and **26**, and enclosed by the outer wall. The fibres are passed through the chambers by way of holes provided in the walls **25**, **25'** and **26**. In the setting chamber **D** and the drying chamber **E**, holes **52** and **53** communicating with a conventional solvent-removal device are provided in the upper parts, and ventilation holes **54**, **55** and **56** and **57** are provided in the bottom of the drafting chamber, the steaming chamber and the drying chamber and the upper part of the wall between the drafting chamber and the steaming chamber.

15 A cooler **F** having a funnel-like section is positioned after the drying chamber **E**. It is provided with an endless belt **60** passing over rollers **58** and **59**, and the fibres **W** passing over the belt **60** are cooled by air drawn through the belt by a suction pipe **61**, and are 20 then introduced into a can by a pair of forwarding rollers **62**.

In the indirect crimping method the treated fibres are further processed by conventional methods and pass to spinning apparatus and dyeing and finishing apparatus, 25 and can optionally be knitted into a fabric using a conventional knitting machine. As a device for stress-releasing the fibres in yarn form there may be used a conventional hank washing machine, hank dyeing machine or a steam box. For knitted fabrics a conventional paddle dyeing machine, a Hofmann press or a winch dyeing machine can be used.

Keratin fibres can be impregnated rapidly and uniformly with an impregnating liquid in the vacuum padder **A** illustrated in FIG. 1 and then pass to the U-type storage duct **B** in FIG. 2, in which they are allowed to stand for 5–10 minutes to allow penetration of the liquid into the fibres.

The fibres are passed to the drafting chamber **C** by way of the tension adjusting rollers **33**, **34** and **35**, and are forwarded to the pair of grip rollers **38** and **39**. The spacing of the grip rollers is adjusted, depending on the average length of fibres to be treated, and the rate of surface speed of the pair of grip rollers **39** is controlled to be 1.0–1.3 times as fast as that of the pair of rollers **38**, so as to draft the fibres. The rate and the amount of drafting depend on the treating method to be employed later, as described previously. In the direct crimping method, the surface speed of the rollers **40** is adjusted to be the same as that of the rollers **38** so that the fibres are overfed by the rollers **39** and become crimped. The fibres are then forwarded to the steaming chamber **D** and remain for 30–60 seconds under no applied tension. A steam jet is directed from the pipe **50** against the fibres through the mesh belt **44** to evaporate the impregnating liquid and set the fibres at 80°–125°C. The evaporated impregnating liquid is discharged out of the exhaust hole **52** to a collector and there collected for re-use. The fibres are then introduced into the drying chamber, wherein they are dried under no applied tension for 30–60 seconds at 80°–110°C to evaporate completely the remaining volatile impregnating liquid. Then, the fibres are forwarded to the cooler **F** to be cooled.

65 In the indirect crimping method, the endless mesh belts **48** and **48'** positioned above the rollers in the steaming set chamber **D** and the drying chamber **E** are both lowered to co-operate with the lower endless belts

44 and 44', so as to maintain drafting forces on the fibres in the drafting chamber. The fibres are drafted with a small amount of drafting, usually 5 - 20 percent but more especially less than 10 percent by adjusting each pair of rollers and the fibres remain under tension while passing through the steaming chamber D and the drying chamber E. The fibres passing through between the endless belts 44 and 48 are contacted with steam from steam jets 50 in the steam setting chamber D for 30 - 60 seconds, to evaporate the volatile impregnating liquid and temporarily set the fibres at 80° - 125°C. Then they are dried in the drying chamber E at 80° - 110°C for 30 - 60 seconds, also under tension, to complete the evaporation of the volatile liquid and this is followed by cooling by the cooler F.

The fibres can subsequently be sent to a gill and then spun into yarns on a conventional spinning machine. Yarns or textile fabrics produced from the yarns can be treated in dyeing and finishing apparatus using steam or boiling water as a medium, for 30 - 60 seconds in the case of yarns and for 10 - 20 minutes in the case of textile fabrics. Then, they can be dried and cooled to produce crimps and bulked spun yarns or textiles obtained having a good handle. If necessary they may be treated with the impregnating liquid described above after the above-described treatment.

The invention is further illustrated by the following Examples.

#### EXAMPLE 1

Australian merino 64'S wool top of 20 g/m, 21.22mm, mean fibre length 75.84 mm. and oil content of 0.68 percent was immersed in the following impregnating liquid:

|                             |               |
|-----------------------------|---------------|
| water                       | 50% by volume |
| n-propanol                  | 47%           |
| formaldehyde solution (40%) | 3%            |

The top was then squeezed to 84 percent wet pick-up by the vacuum padder and allowed to stand for 5 minutes at room temperature. It was drafted to 30 percent extension at room temperature using a grip roller spacing of 76 mm, and the tension was released at room temperature to produce crimp waves. The crimped top was then set by steam at 2 kg/cm<sup>2</sup> pressure, while maintaining an ambient temperature of 120°C, for 30 seconds without applied tension and dried with an indirect heater at 105°C for 60 seconds without applied tension. The crimped fibres exhibited 7 crimps/4 cm as shown in FIG. 3. The top treated by the above crimping method was wound round a glass bar and exposed to boiling water for 10 minutes, but crimp waves still remained.

#### EXAMPLE 2

By the same treatment as described in Example 1, except that drafting ratios of 10 percent and 20 percent respectively were used, there were obtained crimp waves of 5 crimps/4 cm fibre and 6 crimps/4cm fibre. The crimped top was wound round a glass bar and treated in boiling water for 10 minutes, but the crimps were not removed by this treatment.

#### EXAMPLE 3

The same treatment as described in Example 1 was employed, except that the impregnating solution composition was as follows:

|                 |               |
|-----------------|---------------|
| water           | 50% by volume |
| n-propanol      | 45%           |
| 86% formic acid | 5% by volume  |
| pH              | 2.5           |

There were obtained 8 crimps/4 cm fibre. The crimped top was treated in boiling water for 10 minutes, and crimp waves of longer frequency, namely 4 crimps/4 cm fibre, were obtained.

#### EXAMPLE 4

Australian merino 50'S wool top of 20 g/m, 34.77μ, mean fibre length, 199.69 mm and oil content 0.60 was immersed in a solution having the following composition, squeezed to 80 percent pick-up with a mangle and allowed to stand at room temperature for 5 minutes:

|              |               |
|--------------|---------------|
| water        | 50% by volume |
| n-propanol   | 47% do.       |
| formaldehyde | 3% do.        |

After the impregnated top had been allowed to stand, it was drafted to an extension of 30 percent with grip roller spacing of about 120 mm, which equalled the mean fibre length, at room temperature. The drafted top was then quickly released from drafting to produce crimp waves and was steamed with 2 kg/cm<sup>2</sup> steam, in a chamber maintained by an indirect heater at 120°C, for 30 seconds without applied tension to set the fibres, and was then dried at 105°C for 60 seconds without applied tension. There were obtained 7 crimps/6 cm fibre. The crimped top was wound round a glass bar and exposed to boiling water for 10 minutes, but the crimp waves were not eliminated.

#### EXAMPLE 5

Australian merino 65'S top of 20 g/m mean fibre length 75.00 mm 21.14μ and oil content 0.26, and having received an anti-shrinking treatment with 4.5 percent on the fibre weight of sodium dichloroisocyanate, was immersed in a solution of the following composition, squeezed to 80 percent pick-up with a pad mangle and allowed to stand at room temperature for 5 minutes:

|                 |               |
|-----------------|---------------|
| water           | 50% by volume |
| n-propanol      | 47% by volume |
| 86% formic acid | 3% by volume  |
| pH              | 2.5           |

After being allowed to stand, the top was drafted to 20 percent extension with a grip roller spacing of 75 mm (the mean fibre length) and then relaxed quickly from drafting at room temperature to produce crimp waves. The crimp top was steamed at 3 kg/cm<sup>2</sup> pressure for 30 seconds and at a temperature of 125°C, maintained by an indirect heater, without applied tension and dried at 105°C for 60 seconds without applied tension. There were obtained 8 crimps/4 cm fibre. The crimped top was treated with boiling water for 10 minutes without tension, and crimp waves were not removed by this treatment.

## EXAMPLE 6

Australian merino 64'S top of 20 g/m, mean fibre length 75.84 mm 21.22 $\mu$  mean fibre diameter and oil content 0.68 was immersed in a solution of the following composition, squeezed with a mangle to 84 percent wet pick-up and allowed to stand at room temperature for 5 minutes:

|                 |               |
|-----------------|---------------|
| water           | 50% by volume |
| n-propanol      | 47% by volume |
| 28% formic acid | 3% by volume  |
| pH              | 2.5           |

After being allowed to stand, the top was drafted to 10 percent extension at room temperature with a grip roller spacing equal to the mean fibre length, 76 mm, steamed at 3 kg/cm<sup>2</sup> pressure and a temperature of 125°C, maintained by an indirect heater, for 60 seconds under tension, dried at 105°C for 60 seconds under tension, and cooled and wound up directly to a gill ball. The top was spun to yarn of one forty-eighth metre and treated in a conventional hank dyeing machine in boiling water for 10 minutes. Bulked yarns having good handle were obtained.

## EXAMPLE 7

By the same treatment as described in Example 1 was employed, except that the impregnating solution composition was as follows:

|              |                 |
|--------------|-----------------|
| water        | 50 % by volume  |
| iso-propanol | 49.9% by volume |
| 28% ammonia  | 0.1% by volume  |
| pH           | 10.5            |

There were obtained 10 crimps/4 cm fibre, the crimped top was treated with boiled water for 10 minutes, and there were obtained 8 crimps/4 cm fibre.

## EXAMPLE 8

By the same treatment as described in Example 1 was employed, except that the impregnating solution composition was as follows:

|                    |               |
|--------------------|---------------|
| water              | 50% by volume |
| iso-propanol       | 47% do.       |
| thioglycollic acid | 3% do.        |

There were obtained 8 crimps/4 cm fibre. The crimped top was treated with boiled water for 30 minutes and there were obtained 8 crimps/4 cm fibre.

## EXAMPLE 9

By the same treatment as described in Example 1 was employed, except that the impregnating solution composition was as follows:

|                  |      |             |
|------------------|------|-------------|
| water            | 50   | % by volume |
| iso-propanol     | 49.9 | % by volume |
| 28% ammonia      | 0.1  | % by volume |
| thiourea dioxide | 3    | % o.w.f.    |

There were obtained whiter and brighter wool composed of 10 crimps/4 cm fibre. The crimped top was treated with boiled water for 30 minutes and there were obtained 10 crimps/4 cm fibre.

We claim:

1. A method of crimping protein fibres comprising the steps of: applying to said fibres an aqueous solution containing at least 10 percent by volume of an alcohol; drafting said fibres; and releasing said drafting forces applied to said fibres whereby said fibres become crimped.

2. A method according to claim 1 including the additional steps of: setting the crimps in said crimped fibres; and drying said fibres.

3. A method according to claim 1, wherein said aqueous solution applied to said fibres additionally comprises an acid.

4. A method according to claim 3, wherein said acid has a boiling point below 120°C.

5. A method according to claim 1, wherein said aqueous solution additionally comprises formic or acetic acid.

6. A method according to claim 1, wherein said aqueous solution applied to said fibres additionally comprises an alkali.

7. A method according to claim 1, wherein said aqueous solution additionally comprises ammonia.

8. A method according to claim 1, wherein said alcohol has a boiling point below 120°C.

9. A method according to claim 1, wherein said alcohol is selected from the group consisting of n-propanol and isopropanol.

10. A method according to claim 1, wherein said alcohol is selected from the group consisting of methanol, ethanol, n-butanol and isobutanol.

11. A method according to claim 1, wherein said impregnating solution additionally comprises a setting agent for said fibres.

12. A method according to claim 11, wherein said setting agent is selected from the group consisting of thioglycollic acid, monoethanolamine sulphite and bisulphite and thiourea dioxide.

13. A method according to claim 1, wherein said impregnating solution additionally comprises a cross-linking agent for said fibres.

14. A method according to claim 13, wherein said cross-linking agent comprises formaldehyde.

15. A method according to claim 1, wherein said fibres after impregnation with said solution are allowed to stand prior to drafting to allow said solution to penetrate into said fibres.

16. A method according to claim 1, wherein said fibres are drafted by applying drafting forces at at least two points spaced apart by the average fibre length.

17. A method according to claim 1, wherein said fibres are extended during drafting by about 10 - 30 percent.

18. A method according to claim 1, wherein said fibres are in a form selected from the group consisting of carded slivers, tops and rovings in which said fibres are nontwisted and arranged uniformly parallel along the axis of said fibres.

19. A method of crimping protein fibres comprising the steps of: applying to said fibres an aqueous solution containing at least 10 percent by volume of an alcohol; drafting said fibres; setting said fibres while maintaining drafting forces on said fibres; drying said fibres; and subsequently relaxing said fibres whereby said fibres become crimped.

20. A method according to claim 19, wherein said drafted and set fibres are formed into a yarn and said fibres in said yarn are subsequently relaxed.

21. A method according to claim 19, wherein said drafted and set fibres are formed into a yarn, said yarn is formed into a fabric, and said fibres in said fabric are subsequently relaxed.

\* \* \* \* \*